



US008690309B2

(12) **United States Patent**  
McConville et al.

(10) **Patent No.:** US 8,690,309 B2  
(45) **Date of Patent:** \*Apr. 8, 2014

(54) **PRINT PROCESS FOR PHASE SEPARATION INK**

(75) Inventors: **Paul McConville**, Webster, NY (US);  
**Joanne L. Lee**, Rochester, NY (US);  
**Peter G. Odell**, Mississauga (CA);  
**Sandra J. Gardner**, Oakville (CA)

(73) Assignee: **Xerox Corporation**, Norwalk, CT (US)

(\*) Notice: Subject to any disclaimer, the term of this patent is extended or adjusted under 35 U.S.C. 154(b) by 413 days.

This patent is subject to a terminal disclaimer.

(21) Appl. No.: **13/095,038**

(22) Filed: **Apr. 27, 2011**

(65) **Prior Publication Data**

US 2012/0274716 A1 Nov. 1, 2012

(51) **Int. Cl.**

*B41J 2/01* (2006.01)  
*B41J 11/00* (2006.01)  
*B41J 2/005* (2006.01)  
*B41J 2/21* (2006.01)

(52) **U.S. Cl.**

CPC *B41J 2/01* (2013.01); *B41J 11/002* (2013.01);  
*B41J 11/0015* (2013.01); *B41J 2/0057*  
(2013.01); *B41J 2/2107* (2013.01)

USPC ..... **347/101**; 347/102; 347/103; 347/100

(58) **Field of Classification Search**

CPC ..... B41J 2/01; B41J 2/211; B41J 2/1433;  
B41J 2/17; B41J 2/17593; B41J 2/2107;  
B41J 2/1755; B41J 2/2114; B41J 11/0015;  
B41J 2/2056; B41J 2/21; B41J 2/0057;

B41J 11/002  
USPC ..... 347/100, 96, 95, 101, 102, 88, 99, 103,  
347/21, 20; 106/31.6, 31.27, 31.13;  
523/160, 161

See application file for complete search history.

(56) **References Cited**

U.S. PATENT DOCUMENTS

|             |         |                |
|-------------|---------|----------------|
| 4,251,824 A | 2/1981  | Hara et al.    |
| 4,410,899 A | 10/1983 | Haruta et al.  |
| 4,412,224 A | 10/1983 | Sugitani       |
| 4,490,731 A | 12/1984 | Vaught         |
| 4,532,530 A | 7/1985  | Hawkins        |
| 4,601,777 A | 7/1986  | Hawkins et al. |
| 5,195,430 A | 3/1993  | Rise           |

(Continued)

FOREIGN PATENT DOCUMENTS

EP 0 941 855 B1 7/2005

OTHER PUBLICATIONS

Rina Carlini, et al., U.S. Appl. No. 13/095,174, filed Apr. 27, 2011, "Ink Compositions Incorporating Substituted Oxazoline Compounds or Substituted Oxazoline Derivatives," not yet published, 81 pages.

(Continued)

*Primary Examiner* — Manish S Shah

(74) *Attorney, Agent, or Firm* — Marylou J. Lavoie

(57) **ABSTRACT**

A process including disposing at least one phase separation ink in an imagewise fashion onto a final image receiving substrate to form an ink image, wherein disposing is at a first temperature at which the at least one phase separation ink is in a molten, unseparated state; cooling the ink image to a second temperature sufficient to initiate crystallization of at least one component of the at least one phase separation ink, wherein at the second temperature the at least one phase separation ink comprises a crystalline phase and an amorphous phase; wherein the amorphous phase of the at least one phase separation ink substantially penetrates into the final image receiving substrate; and wherein the crystalline phase of the at least one phase separation ink substantially remains on the surface of the final image receiving substrate; applying pressure to the ink image on the final image receiving substrate; and allowing the ink to complete crystallization.

**18 Claims, 4 Drawing Sheets**



(56)

## References Cited

## U.S. PATENT DOCUMENTS

|                   |         |                                  |
|-------------------|---------|----------------------------------|
| 5,231,135 A       | 7/1993  | Machell et al.                   |
| 5,372,852 A       | 12/1994 | Titterington et al.              |
| 5,389,958 A       | 2/1995  | Bui et al.                       |
| 5,621,022 A       | 4/1997  | Jaeger et al.                    |
| 5,698,017 A       | 12/1997 | Sacripante et al.                |
| 5,817,169 A *     | 10/1998 | Sacripante et al. .... 106/31.43 |
| 6,221,137 B1      | 4/2001  | King et al.                      |
| 6,472,523 B1      | 10/2002 | Banning et al.                   |
| 6,476,219 B1      | 11/2002 | Duff et al.                      |
| 6,547,380 B2      | 4/2003  | Smith et al.                     |
| 6,576,747 B1      | 6/2003  | Carlini et al.                   |
| 6,576,748 B1      | 6/2003  | Carlini et al.                   |
| 6,590,082 B1      | 7/2003  | Banning et al.                   |
| 6,646,111 B1      | 11/2003 | Carlini et al.                   |
| 6,663,703 B1      | 12/2003 | Wu et al.                        |
| 6,673,139 B1      | 1/2004  | Wu et al.                        |
| 6,682,587 B2      | 1/2004  | Hendricks et al.                 |
| 6,696,552 B2      | 2/2004  | Mayo et al.                      |
| 6,713,614 B2      | 3/2004  | Carlini et al.                   |
| 6,726,755 B2      | 4/2004  | Titterington et al.              |
| 6,755,902 B2      | 6/2004  | Banning et al.                   |
| 6,821,327 B2      | 11/2004 | Jaeger et al.                    |
| 6,958,406 B2      | 10/2005 | Banning et al.                   |
| 7,053,227 B2      | 5/2006  | Jaeger et al.                    |
| 7,084,190 B2      | 8/2006  | Everhardus et al.                |
| 7,271,284 B2      | 9/2007  | Toma et al.                      |
| 7,381,831 B1      | 6/2008  | Banning et al.                   |
| 7,427,323 B1      | 9/2008  | Birau et al.                     |
| 2011/0059233 A1   | 3/2011  | Liu et al.                       |
| 2012/0274698 A1 * | 11/2012 | Morimitsu et al. .... 347/20     |
| 2012/0274713 A1 * | 11/2012 | Odell et al. .... 347/99         |

## OTHER PUBLICATIONS

Rina Carlini, et al., U.S. Appl. No. 13/095,221, filed Apr. 27, 2011, "Substituted Oxazoline Compounds or Substituted Oxazoline Derivatives," not yet published, 88 pages.

Kentaro Morimitsu, et al., U.S. Appl. No. 13/095,795, filed Apr. 27, 2011, "Solid Ink Compositions Comprising Amorphous Esters of Citric Acid," not yet published, 28 pages.

Peter G. Odell, et al., U.S. Appl. No. 13/095,043, filed Apr. 27, 2011, "Solventless Reaction Process," not yet published, 67 pages.

Naveen Chopra, et al., U.S. Appl. No. 13/095,555, filed Apr. 27, 2011, "Phase Change Inks and Methods of Making the Same," not yet published, 37 pages.

Jennifer L. Belelie, et al., U.S. Appl. No. 13/095,591, filed Apr. 27, 2011, "Phase Change Ink Components and Methods of Making the Same," not yet published, 31 pages.

Kentaro Morimitsu, et al., U.S. Appl. No. 13/095,784, filed Apr. 27, 2011, "Solid Ink Compositions Comprising Amorphous Esters of Tartaric Acid," not yet published, 31 pages.

Kentaro Morimitsu, et al., U.S. Appl. No. 13/095,715, filed Apr. 27, 2011, "Solid Ink Compositions Comprising Crystalline Esters of Tartaric Acid," not yet published, 29 pages.

Kentaro Morimitsu, et al., U.S. Appl. No. 13/095,770, filed Apr. 27, 2011, "Phase Change Inks and Methods of Making the Same," not yet published, 34 pages.

Jennifer L. Belelie, et al., U.S. Appl. No. 13/095,681, filed Apr. 27, 2011, "Solid Ink Compositions Comprising Crystalline-Amorphous Mixtures," not yet published, 31 pages.

Jennifer L. Belelie, et al., U.S. Appl. No. 13/095,636, filed Apr. 27, 2011, "Solid Ink Compositions Comprising Crystalline-Amorphous Mixtures," not yet published, 24 pages.

Kentaro Morimitsu, et al., U.S. Appl. No. 13/095,028, filed Apr. 27, 2011, "Phase Change Ink," not yet published, 39 pages.

Thomas Edward Enright, et al., U.S. Appl. No. 13/095,015, filed Apr. 27, 2011, "Solventless Reaction Process," not yet published, 34 pages.

Marcel Slot, "Oce Printhead and CrystalPoint™ Technology," 16<sup>th</sup> Annual European Inkjet Conference, Nov. 13, 2008, 49 pages.

\* cited by examiner



FIG. 1



FIG. 2



FIG. 3

MICROSCOPY IMAGING OF DTP PRINTS  
PAPER TEMP= ~55°C



FIG. 4

MICROSCOPY IMAGING OF DTP PRINTS  
PAPER TEMP= ~55°C



FIG. 5

**PRINT PROCESS FOR PHASE SEPARATION  
INK**

**RELATED APPLICATIONS**

Commonly assigned U.S. patent application Ser. No. 13/095,174, entitled "Next-Generation Solid Inks From Novel Oxazoline Components, Developed for Robust Direct-to-Paper Printing", filed concurrently herewith, is hereby incorporated by reference herein in its entirety.

Commonly assigned U.S. patent application Ser. No. 13/095,221, entitled "Oxazoline Derivatives: Novel Components for a Next-Generation Robust Solid Ink", filed concurrently herewith, is hereby incorporated by reference herein in its entirety.

Commonly assigned U.S. patent application Ser. No. 13/095,795, entitled "Solid Ink Compositions Comprising Amorphous Esters of Citric Acid", filed concurrently herewith, is hereby incorporated by reference herein in its entirety.

Commonly assigned U.S. patent application Ser. No. 13/095,555, entitled "Phase Change Inks and Methods of Making the Same", filed concurrently herewith, is hereby incorporated by reference herein in its entirety.

Commonly assigned U.S. patent application Ser. No. 13/095,591, entitled "Phase Change Ink Components and Methods of Making the Same", filed concurrently herewith, is hereby incorporated by reference herein in its entirety.

Commonly assigned U.S. patent application Ser. No. 13/095,784, entitled "Solid Ink Compositions Comprising Amorphous Esters of Tartaric Acid", filed concurrently herewith, is hereby incorporated by reference herein in its entirety.

Commonly assigned U.S. patent application Ser. No. 13/095,715, entitled "Solid Ink Compositions Comprising Crystalline Esters of Tartaric Acid", filed concurrently herewith, is hereby incorporated by reference herein in its entirety.

Commonly assigned U.S. patent application Ser. No. 13/095,770, entitled "Phase Change Inks and Methods of Making the Same", filed concurrently herewith, is hereby incorporated by reference herein in its entirety.

Commonly assigned U.S. patent application Ser. No. 13/095,681, entitled "Solid Ink Compositions Comprising Crystalline-Amorphous Mixtures", filed concurrently herewith, is hereby incorporated by reference herein in its entirety.

Commonly assigned U.S. patent application Ser. No. 13/095,636, entitled "Solid Ink Compositions Comprising Crystalline-Amorphous Mixtures", filed concurrently herewith, is hereby incorporated by reference herein in its entirety.

Commonly assigned U.S. patent application Ser. No. 13/095,015, entitled "Solventless Reaction Process", filed concurrently herewith, is hereby incorporated by reference herein in its entirety.

**BACKGROUND**

Disclosed herein is a process comprising disposing at least one phase separation ink in an imagewise fashion onto a final image receiving substrate to form an ink image, wherein disposing is at a first temperature at which the at least one phase separation ink is in a molten, unseparated state; cooling the ink image to a second temperature sufficient to initiate crystallization of at least one component of the at least one phase separation ink, wherein at the second temperature the at least one phase separation ink comprises a crystalline phase and an amorphous phase; wherein the amorphous phase of the at least one phase separation ink substantially penetrates into the final image receiving substrate; and wherein the crystalline phase of the at least one phase separation ink substan-

tially remains on the surface of the final image receiving substrate; applying pressure to the ink image on the final image receiving substrate; and allowing the ink to complete crystallization.

5 Ink jetting devices are known in the art, and thus extensive description of such devices is not required herein. As described in U.S. Pat. No. 6,547,380, which is hereby incorporated by reference herein in its entirety, ink jet printing systems generally are of two types: continuous stream and drop-on-demand. In continuous stream ink jet systems, ink is emitted in a continuous stream under pressure through at least one orifice or nozzle. The stream is perturbed, causing it to break up into droplets at a fixed distance from the orifice. At the break-up point, the droplets are charged in accordance with digital data signals and passed through an electrostatic field that adjusts the trajectory of each droplet in order to direct it to a gutter for recirculation or a specific location on a recording medium. In drop-on-demand systems, a droplet is expelled from an orifice directly to a position on a recording medium in accordance with digital data signals. A droplet is not formed or expelled unless it is to be placed on the recording medium.

10 There are at least three types of drop-on-demand ink jet systems. One type of drop-on-demand system is a piezoelectric device that has as its major components an ink filled channel or passageway having a nozzle on one end and a piezoelectric transducer near the other end to produce pressure pulses. Another type of drop-on-demand system is 15 known as acoustic ink printing wherein an acoustic beam exerts a radiation pressure against objects upon which it impinges. Thus, when an acoustic beam impinges on a free surface such as at the liquid/air interface of a pool of liquid from beneath, the radiation pressure which it exerts against the surface of the pool may reach a sufficiently high level to release individual droplets of liquid from the pool, despite the restraining force of surface tension. Focusing the beam on or near the surface of the pool intensifies the radiation pressure it exerts for a given amount of input power. Still another type 20 of drop-on-demand system is known as thermal ink jet, or bubble jet, and produces high velocity droplets. The major components of this type of drop-on-demand system are an ink filled channel having a nozzle on one end and a heat generating resistor near the nozzle. Printing signals representing 25 digital information originate an electric current pulse in a resistive layer within each ink passageway near the orifice or nozzle, causing the ink vehicle (usually water) in the immediate vicinity to vaporize almost instantaneously and create a bubble. The ink at the orifice is forced out as a propelled droplet as the bubble expands.

30 In a typical design of a piezoelectric ink jet device utilizing phase change or solid inks printing directly on a substrate or on an intermediate transfer member, such as the one described in U.S. Pat. No. 5,372,852, which is hereby incorporated by 35 reference herein in its entirety, the image is applied by jetting appropriately colored inks during four to eighteen rotations (incremental movements) of a substrate (an image receiving member or intermediate transfer member) with respect to the ink jetting head, i.e., there is a small translation of the print 40 head with respect to the substrate in between each rotation. This approach simplifies the print head design, and the small movements ensure good droplet registration. At the jet operating temperature, droplets of liquid ink are ejected from the printing device and, when the ink droplets contact the surface 45 of the recording substrate, either directly or via an intermediate heated transfer belt or drum, they quickly solidify to 50 form a predetermined pattern of solidified ink drops.

Thermal ink jet processes are well known and are described, for example, in U.S. Pat. Nos. 4,601,777, 4,251,824, 4,410,899, 4,412,224 and 4,532,530, the disclosures of each of which are hereby totally incorporated herein.

As noted, ink jet printing processes may employ inks that are solid at room temperature and liquid at elevated temperatures. Such inks may be referred to as hot melt inks or phase change inks. For example, U.S. Pat. No. 4,490,731, which is hereby incorporated by reference herein in its entirety, discloses an apparatus for dispensing solid ink for printing on a substrate such as paper. In thermal ink jet printing processes employing hot melt inks, the solid ink is melted by the heater in the printing apparatus and utilized (i.e., jetted) as a liquid in a manner similar to that of conventional thermal ink jet printing. Upon contact with the printing substrate, the molten ink solidifies rapidly, enabling the colorant to substantially remain on the surface of the substrate instead of being carried into the substrate (for example, paper) by capillary action, thereby enabling higher print density than is generally obtained with liquid inks. Advantages of a phase change ink in ink jet printing are thus elimination of potential spillage of the ink during handling, a wide range of print density and quality, minimal paper cockle or distortion, and enablement of indefinite periods of nonprinting without the danger of nozzle clogging, even without capping the nozzles.

Solid inks for piezoelectric ink jet printing have been designed to successfully print in a transfix mode wherein the ink is jetted onto an intermediate transfer drum. In the transfix printing process, the ink cools from the jetting temperature (broadly, from about 75° C. and to no higher than about 180° C., and typically from about 110° C. to about 140° C.) to the drum temperature (typically from about 50° C. to about 60° C.), and, subsequently, as a substantially solid phase, the ink is pressed into a paper substrate. Such a process provides a number of advantages including vivid images, economy of jet use, and substrate latitude among porous papers. However, such ink designs can present problems when applied to coated papers. In general, the ink and the print process can fail to provide sufficient image durability in response to paper handling stresses such as scratch, fold and rub stresses. Moreover, key elements of the ink design that provide good transfix behavior may not be required or desired in a direct to paper architecture.

Currently available phase change or solid ink printing processes are suitable for their intended purposes. However, a need remains for a printing process providing improved properties including improved adherence of image to paper, improved image permanence, improved robustness against mechanical stresses, and improved image characteristics including surface gloss level. Further, a need remains for a direct to paper printing process for phase separation inks.

The appropriate components and process aspects of the each of the foregoing U.S. Patents and Patent Publications may be selected for the present disclosure in embodiments thereof. Further, throughout this application, various publications, patents, and published patent applications are referred to by an identifying citation. The disclosures of the publications, patents, and published patent applications referenced in this application are hereby incorporated by reference into the present disclosure to more fully describe the state of the art to which this invention pertains.

## SUMMARY

Described is a process comprising disposing at least one phase separation ink in an imagewise fashion onto a final image receiving substrate to form an ink image, wherein

disposing is at a first temperature at which the at least one phase separation ink is in a molten, unseparated state; cooling the ink image to a second temperature sufficient to initiate crystallization of at least one component of the at least one phase separation ink, wherein at the second temperature the at least one phase separation ink comprises a crystalline phase and an amorphous phase; wherein the amorphous phase of the at least one phase separation ink substantially penetrates into the final image receiving substrate; and wherein the crystalline phase of the at least one phase separation ink substantially remains on the surface of the final image receiving substrate; applying pressure to the ink image on the final image receiving substrate; and allowing the ink to complete crystallization.

Also described is a process which comprises (1) incorporating into an ink jet printing apparatus at least one phase separation ink; (2) heating the at least one phase separation ink to a first temperature at which the at least one phase separation ink is in a molten, unseparated state; (3) causing droplets of the at least one phase separation ink to be ejected in an imagewise pattern onto an image receiving substrate, wherein the image receiving substrate is an intermediate transfer member or a final image receiving substrate; (4) cooling the ink image to a second temperature sufficient to initiate crystallization of at least one component of the at least one phase separation ink, wherein the at least one phase separation ink comprises a crystalline phase and an amorphous phase; (5) optionally transferring the ink image from an intermediate transfer member to a final image receiving substrate; wherein the amorphous phase of the at least one phase separation ink substantially penetrates into the final image receiving substrate; and wherein the crystalline phase of the at least one phase separation ink substantially remains on the surface of the final image receiving substrate; (6) applying pressure to the ink image on the final image receiving substrate; and (7) allowing the ink to complete crystallization.

## BRIEF DESCRIPTION OF THE DRAWINGS

FIG. 1 is an illustration of a print process in accordance with the present disclosure.

FIG. 2 is a drawing (left illustration) and a micrograph (right picture) of a printed ink printed in accordance with the present disclosure.

FIG. 3 is a photomicrograph showing a comparative print process (left picture) versus a print process in accordance with the present disclosure (right picture).

FIG. 4 is a photomicrograph showing ink penetration partly into paper top coat but not into paper substrate in accordance with a print process of the present disclosure.

FIG. 5 is a photomicrograph showing no ink penetration into paper top coat or paper substrate in accordance with a comparative print process.

## DETAILED DESCRIPTION

A print process for phase separation ink is described comprising disposing at least one phase separation ink in an imagewise fashion onto an image receiving substrate, in embodiments, onto an intermediate transfer member or directly onto a final image receiving substrate, to form an ink

image, wherein disposing is at a first temperature at which the at least one phase separation ink is in a molten, unseparated state; cooling the ink image to a second temperature sufficient to initiate crystallization of at least one component of the at least one phase separation ink, wherein at the second temperature the at least one phase separation ink comprises a crystalline phase and an amorphous phase; optionally, transferring the ink image to a final image receiving substrate, if required, applying pressure to the ink image on the final image receiving substrate; and allowing the ink to complete crystallization. In embodiments, the process comprises disposing at least one phase separation ink in an imagewise fashion onto a final image receiving substrate to form an ink image, wherein disposing is at a first temperature at which the at least one phase separation ink is in a molten, unseparated state; cooling the ink image to a second temperature sufficient to initiate crystallization of at least one component of the at least one phase separation ink, wherein at the second temperature the at least one phase separation ink comprises a crystalline phase and an amorphous phase; wherein the amorphous phase of the at least one phase separation ink substantially penetrates into the final image receiving substrate; and wherein the crystalline phase of the at least one phase separation ink substantially remains on the surface of the final image receiving substrate; applying pressure to the ink image on the final image receiving substrate; and allowing the ink to complete crystallization.

The process includes employing an ink that can comprise a single phase at jetting temperature and that, upon cooling, can comprise two phases wherein one phase is crystalline and one phase is amorphous, wherein the crystalline phase and has a substantially lower mobility than the separate amorphous phase, and wherein the amorphous phase can penetrate into the image receiving substrate, in embodiments within a top coat layer of a coated paper substrate, while the crystalline phase remains substantially or completely on the top layer without penetration.

The present process can be used for any suitable or desired printing application. In embodiment, the process is a direct printing process wherein one or more phase separation inks are disposed directly onto a final image receiving substrate. In embodiments, the final image receiving substrate is paper. In a direct to paper (DTP) ink jet printing architecture, the ink impacts the paper at essentially the same temperature as the jetting temperature (wherein jetting temperature is typically from about 100° C. to about 140° C.). As the ink cools from the jetting temperature, certain types of ink can phase separate wherein one ink component rapidly crystallizes, while another ink component is in an amorphous state. The amorphous phase continues to penetrate into the paper coating and may carry much of the colorant with it. In this process, the upper layer of crystalline material can act as a less color intensive protective coating that increase resistance of the image to mechanical damage.

The print process herein enables (1) the “molten” state of a single phase separation ink or the “molten” state of two or more inks which become blended color inks in the jetting zone, and (2) the crystallization state of the ink or inks in the spreading zone. The molten and crystallization phases enable print robustness on coated media applications as well as other print quality attributes like uniformity and gloss.

Turning to FIG. 1, a representation of a print process for printing phase separation inks in accordance with the present

disclosure is shown. Print process **10** includes disposing at least one phase separation ink in an imagewise fashion onto a final image receiving substrate **14** to form an ink image **16a**.

Although not limited to any particular order, the process 5 can be described in terms of Steps **1**, **2**, **3**, and **4**, as shown in FIG. 1. In embodiments, the process may include Step **1** comprising jetting one or more phase separation inks from an ink jet print head onto a final ink receiving substrate, in embodiments, paper, in specific embodiments, a coated paper. The temperature of the final image receiving substrate can be higher than the crystallization temperature of the at least one crystalline or crystallizable component in the phase separation ink. Hence, the phase separation ink is in a molten state and is not phase separated in the jetting zone. In embodiments, disposing comprises disposing two or more phase separation inks, optionally of two or more different colors. In other embodiments, disposing comprises ink jetting at least one phase separation ink; and optionally, wherein disposing comprises ink jetting two or more phase separation inks, optionally of two or more different colors. When two or more phase separation inks are disposed, or jetted, blending of inks occurs, such as in the jetting zone.

25 Disposing the at least one phase separation ink can be at any suitable or desired temperature provided that the ink is in a molten, unseparated state. In embodiments, the at least one phase separation ink can be disposed or jetted at a temperature of from about 75 to about 180° C., from about 90 to about 150° C., from about 95° C. to about 140° C., or from about 30 100° C. to about 140° C.

In Step **2**, the process continues along a print process direction indicated by arrow **18** with the movement of the ink image **16a** out of the jetting zone. As the ink image leaves the jetting zone, ink image now designated as **16b**, the ink or inks 35 start to phase separate.

In Step **3**, ink image **16b** continues into a spreading zone. The ink image can be cooled to a second temperature sufficient to initiate or accelerate crystallization of the least one 40 crystalline or crystallizable component of the at least one phase separation ink wherein at the second temperature the at least one phase separation ink comprises a crystalline phase and an amorphous phase. Cooling can be applied first to promote the phase separation of the ink. Cooling can comprise any suitable or desired cooling method. In embodiments, cooling can comprise air cooling, conduction cooling, fluid evaporation cooling, or a combination thereof.

50 Cooling can be to any suitable or desired temperature provided that the temperature is sufficient to initiate crystallization of the least one crystalline or crystallizable component of the at least one phase separation ink. In embodiments, cooling comprises cooling to a second temperature of from about 0 to about 100° C., from about 20 to about 80° C., or from about 25° C. to about 60° C.

55 Referring to Step **3**, in embodiments, cooling can be first applied to the semi-crystallized inks of ink image **16c** in the spreading zone to improve or increase the crystallization rates.

60 After a desired amount of ink separation, which can be determined by any suitable or desired method, such as by measuring temperature and time, pressure can be applied to ink image **16c**, such as with integrated spreader roller **20**. Pressure can be applied to spread the ink and create a desired 65 surface gloss level on the ink image.

Applying pressure can comprise any suitable or desired method to spread the ink on the final image receiving sub-

strate. Applying pressure can further comprise applying any suitable or desired amount of pressure for any suitable or desired amount of time. In embodiments, applying pressure comprises applying pressure of from about 3 to about 5,000 pounds per square inch, from about 100 to about 2,500 pounds per square inch, or from about 500 to about 1,200 pounds per square inch for a period of from about 1 to about 1,000 milliseconds, or from about 3 to about 100 milliseconds, or from about 5 to about 50 milliseconds. In specific embodiments, applying pressure can comprise applying a high pressure of about 100 to about 1,000 pounds per square inch for a period of from about 1 millisecond to about 10 milliseconds.

In embodiments, applying pressure can comprises applying pressure in a manner sufficient to provide the final image with a desired surface gloss. Desired image surface gloss can be any suitable or desired gloss measured by any suitable or desired method. In embodiments, applying pressure comprises applying pressure to spread the ink on the final image receiving substrate in a manner sufficient to provide the final image with a surface gloss of from about 10 to about 50 Gardner 60 degree gloss units at about 60° C.

The process may further comprise employing a release agent to reduce or eliminate ink offset. Any suitable or desired release agent can be selected for the present process. Examples of suitable release agents include, but are not limited to, silicone oil, fountain solution, amine functionalized oils, and combinations thereof.

The release agent can be employed in any suitable or desired amount, such as from about 0.1 to about 50, from about 0.5 to about 20, or from about 1 to about 10 milligrams per A4 size page. In embodiments, when contacting the ink directly in the ink spreading zone, a small amount, such as from about 0.5 milligrams/per A4 size page to about 10 milligrams/per A4 size page of release agent may be used to substantially reduce or eliminate ink offset.

Following the spreader zone, the ink is allowed to fully phase separate and form a robust crystalline surface. Final ink image 16d adheres to the final image receiving substrate and is robust against mechanical stresses such as scratching.

In embodiments, the process comprises controlling the temperature of the final image receiving substrate to control the crystallization rate of the at least one phase separation ink. Controlling the temperature of the final image receiving substrate can be carried out by any suitable or desired method at any suitable or desired time during the process. In embodiments, the final image receiving substrate is paper and the paper temperature is adjusted to keep the inks molten on the paper in the jetting zone. In specific embodiments, the final image receiving substrate is paper and the paper temperature is adjusted to keep the inks molten on the paper in the jetting zone within a range of from about 25° C. to about 85° C. In embodiments, heating the paper can be accomplished before, during, or after disposing the ink.

In another embodiment, the process herein further comprises controlling the temperature of the final image receiving substrate in an ink disposing zone to maintain the temperature of the final image receiving substrate in the ink disposing zone at a temperature that is higher than the crystallization temperature of the at least one phase separation ink, in embodiments, higher than the crystallization temperature of the at least one crystalline or crystallizable component of the phase separation ink. Heating to a temperature that is higher than the crystallization temperature can comprise heating to any suitable or desired temperature that is higher than the crystallization temperature and will depend on the particular materials selected. In embodiments, controlling the tempera-

ture of the final image receiving substrate to maintain the final substrate at a temperature that is higher than the crystallization temperature comprises maintaining the substrate at a temperature of from about 0 to about 150° C., from about 15 to about 100° C., or from about 25° C. to about 60° C.

Controlling the temperature of the final image receiving substrate can be by any suitable or desired method, such as heating. In embodiments, controlling the temperature of the final image receiving substrate in an ink disposing zone to control the crystallization rate of the at least one phase separation ink by heating the final image receiving substrate comprises using infra-red radiation, conductive heating, carrier heating, or a combination thereof.

In embodiments, the ink jetting temperature can be raised to provide a hotter ink than required for simple ink jetting. In embodiments, the process herein comprises disposing the at least one phase separation ink at a third temperature that is higher than the first temperature wherein the third temperature is from about 60 to about 180° C., from about 80 to about 150° C., or from about 45° C. to about 125° C.

Further, the time the ink image resides at a higher temperature can be adjusted to achieve a desired amount of phase separation of multilayers of ink. In embodiments, the process herein further comprises disposing the at least one phase separation ink at a third temperature that is higher than the first temperature at which the at least one phase separation ink is in a molten, unseparated state; and controlling the time that that ink image resides on the final image receiving substrate at the third temperature to achieve a desired amount of phase separation of multilayers of phase separation ink.

Any suitable or desired phase separation ink can be used for the present process. In embodiments, the phase separation ink comprises an ink that is in a molten, unseparated state, that is, a melted, liquid, single phase, at a first temperature corresponding to a disposing or jetting temperature, and that is in a multiple phase state at a second temperature, wherein the second temperature is sufficient to initiate crystallization of at least one component of the phase separation ink, and wherein at the second temperature the phase separation ink comprises a crystalline phase and an amorphous phase. That is, the phase separation ink can comprise at least one component that crystallizes at a second temperature and at least one component that is amorphous at the second temperature.

As used herein, a crystalline component or crystallizable component means a solid material, whose constituent atoms, molecules, or ions are arranged in an orderly repeating pattern extending in all three spatial dimensions.

As used herein, amorphous component means a solid material which does not exhibit crystalline structure. That is, while there may be local ordering of the atoms or molecules, there is no long-term ordering thereof.

The crystalline component selected for embodiments herein can be any suitable or desired crystalline component having the desired characteristics and which is miscible with the selected amorphous component. The crystalline component can have any suitable or desired melting temperature. In embodiments, the crystalline component herein has a melt temperature of from about 65 to about 150° C., from about 66 to about 145° C., or from about 67° C. to about 140° C. In a specific embodiment, the at least one crystalline component herein has a melting temperature less than about 150° C.

The crystalline component can have any suitable or desired crystallization temperature. In embodiments, the crystalline component has a crystallization temperature of from about 60 to about 140° C., from about 65 to about 125° C., or from about 66° C. to about 120° C., as determined by Differential Scanning calorimetry at a rate of 10° C./minute. In a specific

embodiment, the at least one crystalline component herein has a crystallization temperature of greater than about 65° C. to less than about 140° C.

Examples of suitable crystalline or crystallizable components are illustrated in Table 1.

carboxylic acid group or an acid chloride group. Crystalline components are also commercially available, such as from TCI America.

The amorphous components provide tackiness and impart robustness to the printed ink. In the present embodiments,

TABLE 1

| Compound | Structure | T <sub>melt</sub><br>(° C.)* | T <sub>crys</sub><br>(° C.)* | η @ 140° C.<br>(cps)** | η @ RT<br>(cps)**    |
|----------|-----------|------------------------------|------------------------------|------------------------|----------------------|
| 1        |           | 110                          | 83                           | 4.7                    | >10 <sup>6</sup>     |
| 2        |           | 98                           | 71                           | 2.9                    | >10 <sup>6</sup>     |
| 3        |           | 119                          | 80                           | 3.3                    | >10 <sup>6</sup>     |
| 4        |           | 125                          | 75                           | 3.0                    | >10 <sup>6</sup>     |
| Target   |           | <140° C.                     | >65° C.                      | <10 cps                | >10 <sup>6</sup> cps |

\*The samples were measured on a Q1000 Differential Scanning Calorimeter (TA Instruments) at a rate of 10° C./minute from -50° C. to 200° C. to -50° C.; midpoint values are quoted.

\*\*The samples were measured on a RFS3 controlled strain Rheometer (TA Instruments) equipped with a Peltier heating plate and using a 25 millimeter parallel plate. The method used was a temperature sweep from high to low temperatures, in temperature decrements of 5° C., a soak (equilibration) time of 120 seconds between each temperature and at a constant frequency of 1 Hz.

In embodiments, the crystalline component can be crystalline aromatic monoesters described in commonly assigned, co-pending U.S. patent application Ser. No. 13/095,028, which is hereby incorporated by reference herein in its entirety, crystalline diesters described in commonly assigned, co-pending U.S. patent application Ser. No. 13/095,555, which is hereby incorporated by reference herein in its entirety, crystalline esters of tartaric acid as described in co-pending, commonly assigned U.S. patent application Ser. No. 13/095,715, which is hereby incorporated by reference herein in its entirety, and crystalline aromatic amides described in commonly assigned, co-pending U.S. patent application Ser. No. 13/095,770, which is hereby incorporated by reference herein in its entirety.

The crystalline component can be prepared by any suitable or desired method. For example, the crystalline component can be prepared by an esterification reaction between a compound having a hydroxyl group and a compound having a

desirable amorphous materials have relatively low viscosity (<102 cps, or from about 1 to about 100 cps, or from about 5 to about 95 cps) at about 140° C., but very high viscosity (>106 cps) at room temperature. The low viscosity at 140° C. provides wide formulation latitude while the high viscosity at room temperature imparts robustness. The amorphous materials have T<sub>gs</sub> (glass transition temperatures) but do not exhibit crystallization and melting peaks by DSC (10° C./min from -50 to 200 to -50° C.). The T<sub>g</sub> values are typically from about 10 to about 50° C., or from about 10 to about 40° C., or from about 10 to about 35° C., to impart the desired toughness and flexibility to the inks. The selected amorphous materials have low molecular weights, such as less than 1000 g/mol, or from about 100 to about 1000 g/mol, or from about 200 to about 1000 g/mol, or from about 300 to about 1000 g/mol. Higher molecular weight amorphous materials such as polymers become viscous and sticky liquids at high temperatures, but have viscosities that are too high to be jettable with piezoelectric printheads at desirable temperatures. Examples of suitable amorphous materials are illustrated in Table 2.

TABLE 2

| Compound | Structure | Tg<br>(° C.)* | $\eta$ @ 140° C.<br>(cps)** | MW<br>(g/mol) |
|----------|-----------|---------------|-----------------------------|---------------|
| 5        |           | 19            | 10                          | 426.59        |
| 6        |           | 18            | 10                          | 426.59        |
| 7        |           | 13            | 10                          | 426.59        |
| 8        |           | 11            | 27                          | 606.87        |
| Target   |           | 10-50° C.     | <100 cps                    | <1000 g/mol   |

\*The samples were measured on a Q1000 Differential Scanning Calorimeter (TA Instruments) at a rate of 10° C./min from -50° C. to 200° C. to -50° C.; midpoint values are quoted.

\*\*The samples were measured on a RFS3 controlled strain Rheometer (TA instruments) equipped with a Peltier heating plate and using a 25 millimeter parallel plate. The method used was a temperature sweep from high to low temperatures, in temperature decrements of 5° C., a soak (equilibration) time of 120 seconds between each temperature and at a constant frequency of 1 Hz.

In embodiments, the amorphous component can be selected from those described in commonly assigned, co-pending U.S. patent application Ser. No. 13/095,015, which is hereby incorporated by reference herein in its entirety, commonly assigned, co-pending U.S. patent application Ser. No. 13/095,795, which is hereby incorporated by reference herein in its entirety, and commonly assigned, co-pending U.S. patent application Ser. No. 13/095,784, which is hereby incorporated by reference herein in its entirety.

The amorphous component can be prepared by any suitable or desired method. In embodiments, the amorphous component can be prepared as described in commonly assigned, co-pending U.S. patent application Ser. No. 13/095,015, incorporated by reference hereinabove.

The crystalline component can be present in the phase change ink at any suitable or desired amount. In embodi-

ments, the crystalline component is provided at from about 60 to about 95, or from about 65 to about 95, or from about 70 to about 90 weight percent, based upon the total combined weight of the crystalline and amorphous components.

The amorphous component can be present in the phase change ink at any suitable or desired amount. In embodiments, the amorphous component is provided at from about 5 to about 40, or from about 5 to about 35, or from about 10 to about 30 weight percent, based upon the total combined weight of the crystalline and amorphous components.

In embodiments, the ratio of crystalline component to amorphous component is from about 60:40 to about 95:5 percent by weight, based upon the total combined weight of the crystalline and amorphous components. In more specific embodiments, the weight ratio of the crystalline component

to amorphous component is from about 65:35 to about 95:5, or from about 70:30 to about 90:10 percent by weight, based upon the total combined weight of the crystalline and amorphous components.

The phase change inks can further contain a colorant compound. This optional colorant can be present in the ink in any desired or effective amount to obtain the desired color or hue, in embodiments from about 0.1 percent to about 50 percent by weight of the ink. Any desired or effective colorant can be employed, including dyes, pigments, mixtures thereof, and the like, provided that the colorant can be dissolved or dispersed in the ink vehicle. The phase change carrier compositions can be used in combination with conventional phase change ink colorant materials, such as Color Index (C.I.) Solvent Dyes, Disperse Dyes, modified Acid and Direct Dyes, Basic Dyes, Sulphur Dyes, Vat Dyes, and the like.

Examples of suitable dyes include Neozapon® Red 492 (BASF); Orasol® Red G (Pylam Products); Direct Brilliant Pink B (Oriental Giant Dyes); Direct Red 3BL (Classic Dyestuffs); Supranol® Brilliant Red 3BW (Bayer AG); Lemon Yellow 6G (United Chemie); Light Fast Yellow 3G (Shaanxi); Aizen Spilon Yellow C-GNH (Hodogaya Chemical); Bemachrome Yellow GD Sub (Classic Dyestuffs); Cartasol® Brilliant Yellow 4GF (Clariant); Cibanone Yellow 2G (Classic Dyestuffs); Orasol® Black RLI (BASF); Orasol® Black CN (Pylam Products); Savinyl Black RLSN (Clariant); Pyrazol Black BG (Clariant); Morfast® Black 101 (Rohm & Haas); Diaazol Black RN (ICI); Thermoplast® Blue 670 (BASF); Orasol® Blue GN (Pylam Products); Savinyl Blue GLS (Clariant); Luxol Fast Blue MBSN (Pylam Products); Sevron Blue 5GMF (Classic Dyestuffs); Basacid® Blue 750 (BASF); Keyplast Blue (Keystone Aniline Corporation); Neozapon® Black X51 (BASF); Classic Solvent Black 7 (Classic Dyestuffs); Sudan Blue 670 (C.I. 61554) (BASF); Sudan Yellow 146 (C.I. 12700) (BASF); Sudan Red 462 (C.I. 26050) (BASF); C.I. Disperse Yellow 238; Neptune Red Base NB543 (BASF, C.I. Solvent Red 49); Neopen® Blue FF-4012 (BASF); Fastol® Black BR (C.I. Solvent Black 35) (Chemische Fabriek Triade BV); Morton Morplas Magenta 36 (C.I. Solvent Red 172); metal phthalocyanine colorants, such as those disclosed in U.S. Pat. No. 6,221,137, the disclosure of which is totally incorporated herein by reference, and the like. Polymeric dyes can also be used, such as those disclosed in, for example, U.S. Pat. Nos. 5,621,022 and 5,231,135, the disclosures of each of which are hereby incorporated by reference herein in their entireties, and commercially available from, for example, Milliken & Company as Milliken Ink Yellow 869, Milliken Ink Blue 92, Milliken Ink Red 357, Milliken Ink Yellow 1800, Milliken Ink Black 8915-67, uncut Reactint® Orange X-38, uncut Reactint® Blue X-17, Solvent Yellow 162, Acid Red 52, Solvent Blue 44, and uncut Reactint® Violet X-80.

Pigments are also suitable colorants for the phase change inks. Examples of suitable pigments include PALIOGEN® Violet 5100 (BASF); PALIOGEN® Violet 5890 (BASF); HELIOGEN® Green L8730 (BASF); LITHOL® Scarlet D3700 (BASF); SUNFAST® Blue 15:4 (Sun Chemical); Hostaperm® Blue B2G-D (Clariant); Hostaperm® Blue B4G (Clariant); Permanent Red P-F7RK; Hostaperm® Violet BL (Clariant); LITHOL® Scarlet 4440 (BASF); Bon Red C (Dominion Color Company); ORACET® Pink RF (BASF); PALIOGEN® Red 3871 K (BASF); SUNFAST® Blue 15:3 (Sun Chemical); PALIOGEN® Red 3340 (BASF); SUNFAST® Carbazole Violet 23 (Sun Chemical); LITHOL® Fast Scarlet L4300 (BASF); SUNBRITE® Yellow 17 (Sun Chemical); HELIOGEN® Blue L6900, L7020 (BASF); SUNBRITE® Yellow 74 (Sun Chemical); SPECTRA® PAC

C Orange 16 (Sun Chemical); HELIOGEN® Blue K6902, K6910 (BASF); SUNFAST® Magenta 122 (Sun Chemical); HELIOGEN® Blue D6840, D7080 (BASF); Sudan Blue OS (BASF); NEOPEN® Blue FF4012 (BASF); PV Fast Blue B2G01 (Clariant); IRGALITE® Blue GLO (BASF); PALIOGEN® Blue 6470 (BASF); Sudan Orange G (Aldrich); Sudan Orange 220 (BASF); PALIOGEN® Orange 3040 (BASF); PALIOGEN® Yellow 152, 1560 (BASF); LITHOL® Fast Yellow 0991 K (BASF); PALIOTOL® Yellow 1840 (BASF); NOVOPERM® Yellow FGL (Clariant); Ink Jet Yellow 4G VP2532 (Clariant); Toner Yellow HG (Clariant); Lumogen® Yellow D0790 (BASF); Suco-Yellow L1250 (BASF); Suco-Yellow D1355 (BASF); Suco Fast Yellow D1355, D1351 (BASF); HOSTAPERM® Pink E 02 (Clariant); Hansa Brilliant Yellow 5GX03 (Clariant); Permanent Yellow GRL 02 (Clariant); Permanent Rubine L6B 05 (Clariant); FANAL® Pink D4830 (BASF); CINQUASIA® Magenta (DU PONT); PALIOGEN® Black L0084 (BASF); Pigment Black K801 (BASF); and carbon blacks such as REGAL 330™ (Cabot), Nipex 150 (Evonik) Carbon Black 5250 and Carbon Black 5750 (Columbia Chemical), and the like, as well as mixtures thereof.

Pigment dispersions in the ink base may be stabilized by synergists and dispersants. Generally, suitable pigments may be organic materials or inorganic. Magnetic material-based pigments are also suitable, for example, for the fabrication of robust Magnetic Ink Character Recognition (MICR) inks. Magnetic pigments include magnetic nanoparticles, such as for example, ferromagnetic nanoparticles.

Also suitable are the colorants disclosed in U.S. Pat. Nos. 6,472,523, 6,726,755, 6,476,219, 6,576,747, 6,713,614, 6,663,703, 6,755,902, 6,590,082, 6,696,552, 6,576,748, 6,646,111, 6,673,139, 6,958,406, 6,821,327, 7,053,227, 7,381,831 and 7,427,323, the disclosures of each of which are hereby totally incorporated by reference herein in their entireties.

The colorant may be present in the phase change ink in any desired or effective amount to obtain the desired color or hue such as, for example, from about 0.1 to about 50 percent by weight of the ink, about 0.2 to about 20 percent by weight of the ink, or about 0.5 to about 10 percent by weight of the ink.

The inks of the present disclosure can also optionally contain an antioxidant. The optional antioxidants of the ink compositions protect the images from oxidation and also protect the ink components from oxidation during the heating portion of the ink preparation process. Specific examples of suitable antioxidants include NAUGUARD® 524, NAUGUARD® 76, NAUGUARD® 445, and NAUGUARD® 512, commercially available from Uniroyal Chemical Company, Oxford, Conn., IRGANOX® 1010 (Ciba Geigy), N,N'-hexamethylene bis(3,5-di-tert-butyl-4-hydroxy hydrocinnamamide) (IRGANOX® 1098, BASF), 2,2-bis(4-(2-(3,5-di-tert-butyl-4-hydroxyhydrocinnamoyloxy)ethoxyphenyl)propane (TOPANOL-205®, available from Vertellus), tris(4-tert-butyl-3-hydroxy-2,6-dimethyl benzyl)isocyanurate (Aldrich), 2,2'-ethylidene bis(4,6-di-tert-butylphenyl)fluoro phosphonite (ETHANOX-398®, Albermarle Corporation), tetrakis (2,4-di-tert-butylphenyl)-4,4'-biphenyl diphosphonite (ALDRICH 46), pentaerythritol tetrastearate (TCI America), tributylammonium hypophosphite (Aldrich), 2,6-di-tert-butyl-4-methoxyphenol (Aldrich), 2,4-di-tert-butyl-6-(4-methoxybenzyl)phenol (Aldrich), 4-bromo-2,6-dimethylphenol (Aldrich), 4-bromo-3,5-didimethylphenol (Aldrich), 4-bromo-2-nitrophenol (Aldrich), 4-(diethyl aminomethyl)-2,5-dimethylphenol (Aldrich), 3-dimethylaminophenol (Aldrich), 2-amino-4-tert-amylophenol (Aldrich), 2,6-bis(hydroxymethyl)-p-cresol (Aldrich), 2,2'-methylenediphenol

## 15

(Aldrich), 5-(diethylamino)-2-nitrosophenol (Aldrich), 2,6-dichloro-4-fluorophenol (Aldrich), 2,6-dibromo fluoro phenol (Aldrich),  $\alpha$ -trifluoro-o-cresol (Aldrich), 2-bromo-4-fluorophenol (Aldrich), 4-fluorophenol (Aldrich), 4-chlorophenyl-2-chloro-1,1,2-tri-fluoroethyl sulfone (Aldrich), 3,4-difluoro phenylacetic acid (Aldrich), 3-fluorophenylacetic acid (Aldrich), 3,5-difluoro phenylacetic acid (Aldrich), 2-fluorophenylacetic acid (Aldrich), 2,5-bis (trifluoromethyl)benzoic acid (Aldrich), ethyl-2-(4-(4-(trifluoromethyl)phenoxy)phenoxy)propionate (Aldrich), tetrakis(2,4-di-tert-butyl phenyl)-4,4'-biphenyl diphosphonite (Aldrich), 4-tert-amyl phenol (Aldrich), 3-(2H-benzotriazol-2-yl)-4-hydroxy phenethylalcohol (Aldrich), and the like, as well as mixtures thereof. When present, the optional antioxidant is present in the ink in any desired or effective amount, such as from about 0.01 percent to about 20 percent by weight of the ink.

Other optional additives to the inks include defoamer, slip and leveling agents clarifiers, tackifiers, adhesives, plasticizers, and the like, in any suitable or desired amount such as from about 0.1 to about 50 percent by weight of the ink.

The phase change ink can be prepared by any suitable or desired method. For example, the components can be combined with stirring and heating to form the phase change ink. The phase change ink carrier materials may be combined in any suitable or desired order. For example, each of the components of the ink carrier can be mixed together, followed by heating the mixture to at least its melting point, for example from about 60° C. to about 150° C., about 80° C. to about 145° C., or about 85° C. to about 140° C., although not limited. The colorant may be added before the ink ingredients have been heated or after the ink ingredients have been heated. When pigments are the selected colorants, the molten mixture may be subjected to grinding in an attritor or ball mill apparatus or other high energy mixing equipment to affect dispersion of the pigment in the ink carrier. The heated mixture can then be stirred, such as for about 5 seconds to about 30 minutes or more, to obtain a substantially homogeneous, uniform melt, followed by cooling the ink to ambient temperature (typically from about 20° C. to about 25° C.). The inks are solid at ambient temperature.

The ink compositions herein generally have melt viscosities of from about 1 centipoise to about 14 centipoise, or from about 2 centipoise to about 13 centipoise, or from about 3 centipoise to about 12 centipoise, although the melt viscosity can be outside of these ranges, at the jetting temperature, in embodiments, jetting temperature being from about 95° C. to about 150° C., about 100° C. to about 145° C., about 100° C. to about 140° C., or no higher than about 150° C., although the jetting temperature can be outside of these ranges. In embodiments, the phase change ink herein has a viscosity at jetting temperature of from about 2 centipoise to less than about 10 centipoise, wherein jetting temperature is from about 50° C. to about 140° C. In a specific embodiment, the phase change ink herein has a viscosity of less than about 10 centipoise at jetting temperature, wherein jetting temperature is from about 50° C. to about 140° C. In another specific embodiment, the phase change ink herein has a viscosity of about 0.5 to about 10 centipoise at a jetting temperature of about 140° C.

The phase change inks herein can be employed in apparatus for direct printing ink jet processes and in indirect (offset) printing ink jet applications. One embodiment of the present disclosure is directed to a process which comprises incorporating a phase separation ink into an ink jet printing apparatus,

## 16

melting the ink, and causing droplets of the melted ink to be ejected in an imagewise pattern onto a recording substrate. A direct printing process is disclosed in, for example, U.S. Pat. No. 5,195,430, the disclosure of which is totally incorporated herein by reference. In embodiments, the substrate is a final recording sheet and droplets of the melted ink are ejected in an imagewise pattern directly onto the final recording sheet.

Yet another embodiment of the present disclosure is directed to a process which comprises incorporating a phase separation ink into an ink jet printing apparatus, melting the ink, causing droplets of the melted ink to be ejected in an imagewise pattern onto an intermediate transfer member, and transferring the ink in the imagewise pattern from the intermediate transfer member to a final recording substrate. In embodiments, the process can include using a belt or thin drum to transport the ink image on the intermediate transfer member through the temperatures zones necessary to induce the phase separation and then transfer and spread the ink image on a final image receiving substrate. In a specific embodiment, the intermediate transfer member is heated to a temperature above that of the final recording sheet and below that of the melted ink in the printing apparatus. In another specific embodiment, both the intermediate transfer member and the final recording sheet are heated; in this embodiment, both the intermediate transfer member and the final recording sheet are heated to a temperature below that of the melted ink in the printing apparatus; in this embodiment, the relative temperatures of the intermediate transfer member and the final recording sheet can be (1) the intermediate transfer member is heated to a temperature above that of the final recording substrate and below that of the melted ink in the printing apparatus; (2) the final recording substrate is heated to a temperature above that of the intermediate transfer member and below that of the melted ink in the printing apparatus; or (3) the intermediate transfer member and the final recording sheet are heated to approximately the same temperature. An offset or indirect printing process is also disclosed in, for example, U.S. Pat. No. 5,389,958, the disclosure of which is totally incorporated herein by reference. In one specific embodiment, the printing apparatus employs a piezoelectric printing process wherein droplets of the ink are caused to be ejected in imagewise pattern by oscillations of piezoelectric vibrating elements. In embodiments, the intermediate transfer member is heated to a temperature above that of the final recording sheet and below that of the melted ink in the printing apparatus.

Inks of the present disclosure can also be employed in other hot melt printing processes, such as hot melt acoustic ink jet printing, hot melt thermal ink jet printing, hot melt continuous stream or deflection ink jet printing, and the like. Phase change inks of the present disclosure can also be used in printing processes other than hot melt ink jet printing processes.

In embodiments, a process herein comprises (1) incorporating into an ink jet printing apparatus at least one phase separation ink; (2) heating the at least one phase separation ink to a first temperature at which the at least one phase separation ink is in a molten, unseparated state; (3) causing droplets of the at least one phase separation ink to be ejected in an imagewise pattern onto a final image receiving substrate; (4) cooling the ink image to a second temperature sufficient to initiate crystallization of at least one component

of the at least one phase separation ink, wherein the at least one phase separation ink comprises a crystalline phase and an amorphous phase; wherein the amorphous phase of the at least one phase separation ink substantially penetrates into the final image receiving substrate; and wherein the crystalline phase of the at least one phase separation ink substantially remains on the surface of the final image receiving substrate; (5) applying pressure to the ink image on the final image receiving substrate; and (6) allowing the ink to complete crystallization.

In certain embodiments, the process herein comprises disposing at least one phase separation ink in an imagewise fashion onto a final image receiving substrate to form an ink image, wherein the at least one phase separation ink comprises at least one crystalline component selected from the compounds of Table 1 and at least one amorphous component selected from the compounds of Table 2, wherein disposing is at a first temperature at which the at least one phase separation ink is in a molten, unseparated state; cooling the ink image to a second temperature sufficient to initiate crystallization of at least one component of the at least one phase separation ink, wherein at the second temperature the at least one phase separation ink comprises a crystalline phase and an amorphous phase; applying pressure to the ink image on the final image receiving substrate; and allowing the ink to complete crystallization.

Any suitable substrate or recording sheet can be employed, including plain papers such as XEROX® 4200 papers, XEROX® Image Series papers, Courtland 4024 DP paper, ruled notebook paper, bond paper, coated paper, silica coated papers such as Sharp Company silica coated paper, JuJo paper, Hammermill® Laserprint Paper, and the like, glossy coated papers, such as XEROX® Digital Color Elite Gloss, Sappi Warren Papers LUSTROGLOSS®, specialty papers such as Xerox® DURAPAPER®, and the like, calcium carbonate coated paper, clay coated paper, kaolin clay coated paper, and the like, transparency materials, fabrics, textile products, plastics, polymeric films, inorganic substrates such as metals and wood, and the like. In a specific embodiment, the final image receiving substrate is coated paper. In another specific embodiment, the final image receiving substrate is clay coated paper.

In embodiments, the process herein comprises a process wherein the final image receiving substrate comprises a base layer, a top coat layer disposed over a first surface of the base layer; and, optionally, a bottom coat layer disposed over a second, opposite surface of the base layer; wherein the ink image is disposed on the top coat layer; wherein the amorphous phase of the at least one phase separation ink substantially penetrates into the top coat layer of the final image receiving substrate; and wherein the crystalline phase of the at least one phase separation ink substantially remains on the surface of the top coat layer of the final image receiving substrate.

The morphology of the ink image on paper can play a large role in determining the robustness of the image. For instance, an ink that soaks deep into the paper may approach the robustness of the paper itself as it cannot be damaged without damage to the paper itself. However, such an ink may have noticeable and objectionable image show-through on the reverse side of the paper. The present process provides partial penetration of phase separation ink into coated papers. In embodiments, this is accomplished by soaking into the thin coating at the paper surface. The coating in most papers consists of calcium carbonate and/or kaolin clay with a small amount of polymer binder. The process herein provides parameters that favor the crystallization of one ink compo-

5 nent. In some ink formulations, a crystalline material may “super-cool” forming a glass so rapidly that the molecules lack the mobility to crystallize. The present process can comprise maintaining an intermediate temperature at which the molecules have sufficient mobility to crystallize so as to reduce or eliminate this super-cooling effect. Additionally, the amorphous phase that penetrates into the paper coating is generally chosen to have many orders of magnitude variation in viscosity between the jetting temperature and ambient temperature. In embodiments, selected print process temperatures can be selected herein to determine the degree of penetration of the amorphous phase into the paper coating. In specific embodiments, a set of time, temperature, and pressure parameters are selected to provide the desired degree of spreading of the ink image.

## EXAMPLES

The following Examples are being submitted to further define various species of the present disclosure. These Examples are intended to be illustrative only and are not intended to limit the scope of the present disclosure. Also, parts and percentages are by weight unless otherwise indicated.

### Example 1

35 52.4 grams of Compound 3 of Table 1 (above) were combined with 22.5 grams of Compound 6 of Table 2 (above) and stirred at 140° C. for 1 hour. A fine precipitate remained so the ink base was filtered with a 5 µm sieve to form a clear, dark amber solution. To this solution was added 2.3 g Orasol Blue GN (Ciba) and the full ink was stirred for an additional hour 40° C. The ink was filtered easily through a 5 µm sieve.

40 The ink of Example 1 was printed according to the process described herein including steps equivalent steps to FIG. 1. The ink of Example 1 was loaded into a modified Xerox® 8860 printer. The ink was melted at 115° C. and jetted on to glossy paper at 55° C. The paper with jetted ink was transported to a second modified Xerox® 8860 for a spreading process. The printer applied pressure of 800 pounds per square inch at an elevated temperature of 57.5° C. on the ink image at a speed of 1 letter-size paper per second.

45 FIG. 2 provides a schematic illustration (left picture of FIG. 2) and a micrograph (right picture of FIG. 2) of the present print process showing the ink of Example 1 as a cross-sectional image after printing by the present process. The cross-sectional micrograph of FIG. 2, and the remaining micrographs described herein, were taken using an Axialplan optical microscope available from Carl Zeiss, Inc. The schematic illustration is intended as a guide for the eye as the micrograph on the right is examined and shows the penetration of the ink into the paper coating layer.

50 FIG. 3 is a photomicrograph showing a comparative print process (left picture) using a currently available ink (Xerox® Part Number 108R00749) versus a print process in accordance with the present disclosure (right picture) using the present process and an ink as described U.S. patent application Ser. No. 13/095,043, entitled “Phase Separation Ink”, Examples 3a and 3b, General Preparation of Oxazoline Ink, prepared as follows.

19

A. Preparation of Oxazoline Crystalline Phase-Change Component.



20

B. Preparation of Amorphous Binder Resin of Oxazoline Ink.

Step I: Synthesis of Dimer Oxazoline Tetra-Alcohol precursor

5



A 1 Liter Parr reactor equipped with a double turbine agitator, and distillation apparatus, was charged with dodecanoic acid (200 grams; SIGMA-ALDRICH, Milwaukee, Wis.), tris(hydroxymethyl)amino-methane (92 grams; EMD Chemicals, New Jersey), and FASCAT® 4100 as catalyst (0.45 grams; Arkema Inc). The contents were heated to 165° C. for a 2 hour period, followed by increasing the temperature to 205° C. over a 2 hour period during which time the water distillate was collected in a distillation receiver. The reactor pressure was then reduced to about 1-2 mm-Hg for one hour, followed by discharging into a container and cooled to room temperature. The product was purified by dissolving with mild heating in a mixture of ethyl acetate (2.5 parts) and hexane (10 parts), and then cooling to room temperature to crystallize the pure product as a white granular powder. The peak melting point (DSC) was determined to be 99° C. Rheological analysis of this material was measured over a temperature range of 130° C. down to 40° C. using a RFS3 Rheometrics instrument (oscillation frequency of 1 Hz, 25 millimeter parallel plate geometry, 200% applied strain). The material exhibited a melt viscosity at 130° C. of 8.2 cPs, an onset temperature of crystallization at 95° C., a peak viscosity of 4.5×10<sup>6</sup> cPs, and a peak crystallization temperature at 85° C.

20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8

21



-continued

22



Into a 1 liter stainless steel jacketed Buchi reactor equipped with distillation condenser, 4-blade impeller, and thermocouple was charged, in order: 30.4 grams (0.075 mol) Dimer Oxazoline Tetra Alcohol of Step I, 228.2 grams (1.50 mol) 4-methoxybenzoic acid, 51.48 grams (0.425 mol) tris(hydroxymethyl)aminomethane (obtained from Aldrich, 98%), and 0.26 gram (1.2 mmol) FASCAT® 4100 catalyst. The mixture was heated up to 160° C. jacket temperature under a pressurized nitrogen atmosphere of 50 kPa without stirring. Once at temperature, the stirring was begun and the jacket temperature was gradually increased to 180° C. over 30 minutes, and then maintained for about 2 hours. Water distillate from the condensation reaction was collected over this time period (about 10 grams). The jacket temperature was then increased to 190° C. and maintained for 1 hour, which produced more water distillate. Vacuum reduced pressure of ~10 torr was applied for another 1 hour, which produced ~10 grams of water distillate. Once there was no more water distillate collected, the reaction was stopped by cooling to 130° C., and then the product was discharged. The crude yield of resin product was about 400 grams, obtained as a light amber-colored viscous resin without further purification. Rheological analysis of this material was measured over a temperature range of 130° C. down to 40° C. using a RFS3 Rheometrics instrument (oscillation frequency of 1 Hz, 25 mm parallel plate geometry, 200% applied strain). The viscosity of this material at 130° C. was measured to be about 75 cPs, and viscosity of about 1.5×10<sup>5</sup> cPs at about 50° C.

Two example formulations of Oxazoline Inks are provided in Table 3 below.

TABLE 3

|                                | Component                                                                 | Example 3a<br>Wt % | Example 3b<br>Wt % |
|--------------------------------|---------------------------------------------------------------------------|--------------------|--------------------|
| Crystalline Phase-change agent | A<br>Oxazoline Compound                                                   | 62.80              | 63.5               |
| Amorphous Binder Resin         | B<br>Oxazoline Material (KEMAMIDE S-180 (obtained from Witco Corp., USA)) | 30.00              | 30.00              |
| Viscosity modifier             | (KEMAMIDE S-180 (obtained from Witco Corp., USA))                         | 4.00               | 3.50               |
| Antioxidant                    | Naugard 445 (obtained from Chemtura, USA)                                 | 0.20               | 0.00               |
| Colorant                       | Orasol Blue GN dye (obtained from Ciba-Geigy, USA)                        | 3.00               | 3.00               |
| Ink Properties                 | *Viscosity @ 130° C. (cPs)                                                | 13.6               | 11.20              |

TABLE 3-continued

| Component                          | Example 3a<br>Wt %    | Example 3b<br>Wt %    |
|------------------------------------|-----------------------|-----------------------|
| *Viscosity @ 60° C. (cPs)          | 4.6 × 10 <sup>6</sup> | 5.4 × 10 <sup>7</sup> |
| Onset Tcryst. (° C.) (by rheology) | 78                    | 88                    |
| Melt Temp (° C.) (by DSC**)        | 81.5                  | 89                    |
| Tcryst. (° C.) (by DSC**)          | 62 (small)            | 66.5                  |
|                                    | 54 (large)            |                       |

\*Oscillation Frequency = 1 Hz; 25 mm parallel plate geometry; gap = 0.2 mm; strain % = 200%-400%; strain independent viscosities as measured on a Rheometrics RFS3 instrument. \*\*DSC analysis performed on a TA Instruments Q1000 machine, measured after two heating and cooling cycles using a scan rate of 10° C./min.

Into a 500 milliliter resin kettle was charged, in the following order: amorphous oxazoline binder resin prepared according to B, above, (30 weight % of ink); molten oxazoline crystalline compound prepared according to A, above, (62-64 weight % of ink; see formulations in Table 3); Kemamide® S-180 as a viscosity modifier (commercially available from Chemtura Corporation) (3-4 weight % of ink); NAUGARD 445® as antioxidant (obtained from Chemtura, USA); and lastly a colorant (Orasol Blue GN dye, obtained from Ciba-Geigy, USA). The mixture was heated in a mantle at 130° C. internal temperature and stirred mechanically for about 2 hours using a stainless steel 4-blade 90° pitch impeller at approximately 175-250 rpm. The ink base mixture was then hot-filtered at 120° C. using a KST filtration apparatus through a 5-micron stainless steel 325×2300 mesh wire filter cloth (type 304 SS obtained from Gerard Daniel Worldwide, Hanover, USA), in order to remove particulates. The molten mixture was returned to a 500 milliliter resin kettle and heated at 130° C. internal temperature while stirring mechanically. Into this ink base was added colorant (6.0 grams of Orasol® Blue GN dye, obtained from CIBA; 3 weight % of ink) in small portions over a 0.5 hour period of time while continuing to heat. Once the colorant addition was completed, the colored ink composition was allowed to stir for addition 3-4 hrs at 130° C. while stirring at 275 rpm, to ensure homogeneity of the ink composition. The colored ink composition was then hot-filtered once more at 120° C. through the steel 325×2300 mesh wire filter cloth, before being dispensed into mould trays and solidified while cooling at room temperature. The colored ink compositions were characterized for thermal properties by DSC and for rheological properties using the Rheometrics RFS3 strain-controlled rheometer instrument. The ink of Example 3a and the comparative ink were separately loaded into a modified Xerox® 8860 printer. Each ink was melted at 115° C. and jetted on to the DCEG glossy paper

23

at 55° C. The paper with jetted ink was transported to a second modified Xerox® 8860 for a spreading process. The printer applied pressure of 800 pounds per square inch at an elevated temperature of 57.5° C. on the ink image at a speed of 1 letter-size paper per second. The Comparative ink process shown on the left picture of FIG. 3 illustrates that the ink resides on the paper surface. The ink process of the present disclosure shown on the right picture of FIG. 3 illustrates the ink penetration into the top coat layer of the coated paper.

FIG. 4 is a photomicrograph of the ink of Example 3a as described above, disposed in accordance with the present process. FIG. 4 shows ink penetration partly into the paper top coat but not into the paper substrate.

FIG. 5 is a photomicrograph of a printed image prepared with a currently available ink (Xerox® Part Number 108R00749) showing no ink penetration into paper top coat or paper substrate.

In embodiments, it is desired to maintain the molten state of the phase separation inks in the ink spreading zone. An image was printed in accordance with a comparative process wherein a first cyan layer is applied and a second magenta layer is separately applied over the first cyan layer wherein the substrate temperature is maintained at a temperature that is below the crystallization temperature of the magenta and cyan inks. A period of time of about 1 second elapsed between disposing the layers to allow the first ink layer to crystallize before the second ink layer was applied. This induced failure in gouge measurements due to poor ink to ink adhesions. Gouge measurement is a test employing a scratch/gouge finger with a curved tip at an angle of about 15° from vertical, with a weight of 528 grams applied, drawn across the image at a rate of approximately 13 millimeters/second. The scratch/gouge tip is similar to a lathe round nose cutting bit with radius of curvature of approximately 12 millimeters. In a successful ink test, no ink is visibly removed from the image. The upper magenta layer was removed during the gouge test, suggesting that the cyan and magenta inks did not coalesce.

An image was printed wherein a first cyan ink and a second magenta ink are applied simultaneously in a jetting zone onto a substrate with the cyan and magenta inks kept in a molten state, allowed to blend, and then the print imaged cooled so that the inks phase separate in accordance with a process of the present disclosure. This print was robust for gouge measurements. This print appeared more blue in color than the print of the preceding paragraph, suggesting that the two inks had blended. In embodiments herein, the final image printed with the present process shows no visible loss of ink when subjected to a gouge test comprising drawing a gouge finger having a curved tip at an angle of about 15° from vertical with a weight of 528 grams across the final image at a rate of about 13 millimeters per second.

It will be appreciated that various of the above-disclosed and other features and functions, or alternatives thereof, may be desirably combined into many other different systems or applications. Also that various presently unforeseen or unanticipated alternatives, modifications, variations or improvements therein may be subsequently made by those skilled in the art which are also intended to be encompassed by the following claims. Unless specifically recited in a claim, steps or components of claims should not be implied or imported from the specification or any other claims as to any particular order, number, position, size, shape, angle, color, or material.

The invention claimed is:

1. A process comprising:  
disposing at least one phase separation ink in an imagewise fashion onto a final image receiving substrate to form an

24

ink image, wherein disposing is at a first temperature at which the at least one phase separation ink is in a molten, unseparated state;

wherein the at least one phase separation ink comprises at least one crystalline component selected from compounds of the formula



wherein the at least one phase separation ink comprises at least one amorphous component selected from compounds of the formula



25

-continued



cooling the ink image to a second temperature sufficient to initiate crystallization of at least one component of the at least one phase separation ink, wherein at the second temperature the at least one phase separation ink comprises a crystalline phase and an amorphous phase; applying pressure to the ink image on the final image receiving substrate; and allowing the ink to complete crystallization.

2. The process of claim 1, wherein disposing comprises disposing two or more phase separation inks of two or more different colors.

3. The process of claim 1, wherein disposing comprises ink jetting at least one phase separation ink; and

optionally, wherein disposing comprises ink jetting two or more phase separation inks of two or more different colors.

4. The process of claim 1, wherein disposing is at a first temperature of from 100° C. to 140° C.

5. The process of claim 1, wherein cooling comprises cooling to a second temperature of from 20° C. to 80° C.

6. The process of claim 1, wherein applying pressure comprises applying a high pressure of 100 to 1,000 pounds per square inch for a period of from 1 millisecond to 10 milliseconds.

7. The process of claim 1, further comprising:

controlling the temperature of the final image receiving substrate to control the crystallization rate of the at least one phase separation ink.

8. The process of claim 1, further comprising:

controlling the temperature of the final image receiving substrate in an ink disposing zone to maintain the temperature of the final image receiving substrate in the ink disposing zone at a temperature that is higher than the crystallization temperature of the at least one phase separation ink.

9. The process of claim 1, further comprising:

controlling the temperature of the final image receiving substrate in an ink disposing zone to control the crystallization rate of the at least one phase separation ink by heating the final image receiving substrate using infrared radiation, conductive heating, carrier heating, or a combination thereof.

26

10. The process of claim 1, further comprising: disposing the at least one phase separation ink at a third temperature that is higher than the first temperature, wherein the third temperature is from 60° C. to 180° C.

11. The process of claim 1, further comprising: disposing the at least one phase separation ink at a third temperature that is higher than the first temperature at which the at least one phase separation ink is in a molten, unseparated state; and

controlling the time that the ink image resides on the final image receiving substrate at the third temperature to achieve a desired amount of phase separation of multi-layers of phase separation ink.

12. The process of claim 1, wherein the final image receiving substrate is coated paper.

13. The process of claim 1, wherein the final image receiving substrate comprises a base layer, a top coat layer disposed over a first surface of the base layer; and, optionally, a bottom coat layer disposed over a second, opposite surface of the base layer;

wherein the ink image is disposed on the top coat layer.

14. The process of claim 1, further comprising: employing a release agent to reduce or eliminate ink offset.

15. The process of claim 1, wherein the final image shows no visible loss of ink when subjected to a gouge test comprising drawing a gouge finger having a curved tip at an angle of 15° from vertical with a weight of 528 grams across the final image at a rate of 13 millimeters per second.

16. A process which comprises:

(1) incorporating into an ink jet printing apparatus at least one phase separation ink; wherein the at least one phase separation ink comprises at least one crystalline component selected from compounds of the formula



and



and

wherein the at least one phase separation ink comprises at least one amorphous component selected from compounds of the formula

27



28

(2) heating the at least one phase separation ink to a first temperature at which the at least one phase separation ink is in a molten, unseparated state;

5 (3) causing droplets of the at least one phase separation ink to be ejected in an imagewise pattern onto an image receiving substrate, wherein the image receiving substrate is an intermediate transfer member or a final image receiving substrate;

(4) cooling the ink image to a second temperature sufficient to initiate crystallization of at least one component of the at least one phase separation ink, wherein the at least one phase separation ink comprises a crystalline phase and an amorphous phase;

(5) optionally transferring the ink image from an intermediate transfer member to a final image receiving substrate;

(6) applying pressure to the ink image on the final image receiving substrate; and

(7) allowing the ink to complete crystallization.

17. The process of claim 16, further comprising:

controlling the temperature of the final image receiving substrate to control the crystallization rate of the at least one phase separation ink.

18. The process of claim 16, wherein the final image receiving substrate comprises a base layer, a top coat layer disposed over a first surface of the base layer; and, optionally, a bottom coat layer disposed over a second, opposite surface of the base layer;

wherein the ink image is disposed on the top coat layer.

\* \* \* \* \*